

# UNITED STATES PATENT OFFICE.

CHARLES DEAR, OF LONDON, ENGLAND, ASSIGNOR TO THE MIRIS STEEL COMPANY  
LIMITED, OF LONDON, ENGLAND.

## MANUFACTURE OF STEEL.

1,304,948.

Specification of Letters Patent. Patented May 27, 1919.

No Drawing.

Application filed December 30, 1916. Serial No. 139,910.

To all whom it may concern:

Be it known that I, CHARLES DEAR, a subject of the King of England, residing in London, England, have invented certain new and useful Improvements in the Manufacture of Steel, of which the following is a specification.

This invention relates to the manufacture of steel and is of a process to give the steel a treatment whereby a better steel shall result than if the said treatment be not employed.

The present invention provides a process for the treatment of steel by which a freshly-cast ingot is, before its interior is set solid, immersed in water or in an aqueous solution and is kept submerged therein sufficiently long to prevent recalescence of the ingot after it has been removed from the said liquid.

In a modified form of process according to this invention a freshly-cast ingot that has not cooled to a temperature so low as to entirely solidify the interior is immersed in water or an aqueous solution and is kept submerged therein sufficiently long to prevent recalescence after its removal from submersion, for example the ingot may be stripped from the mold or taken from the soaking pit and thus immersed.

Some of the advantages resulting from this invention may be obtained if an ingot above the temperature of recalescence, and before it has been rolled or has otherwise had its surface mechanically worked, is immersed in water or an aqueous solution and kept submerged long enough to prevent recalescence after it has been removed from the said liquid.

In any case the best results are obtained if the solution in which the ingot is immersed be one containing solutes, such as will upon the immersion of the ingot liberate hydrogen at the surface of contact of the ingot with the solution.

It will be understood, therefore, that by this invention an ingot may be plunged either directly the mold has been stripped from it, or alternatively after it has been in the soaking pit for some time, or again alternatively at any time provided its surface has not been mechanically worked, as for example by rolling, and if it be at a temperature above that of recalescence.

The best results, however, are obtained if

the ingot be plunged as soon as practicable after the mold has been stripped from it and while its interior is still fluid or semi-fluid. The sudden contraction of the shell gives rise to a strong compressive action 60 upon the contents of the ingot and it is to this that we attribute some of the beneficial results of the treatment. Other beneficial results follow from the production of hydrogen at the surface of contact of the ingot with the solution; these results are best promoted by employing a solution containing materials which either themselves liberate or promote liberation of hydrogen under the conditions stated. 70

The beneficial results of the treatment are not confined, as might be expected, to a superficial layer of the material, but appear to penetrate so deeply into the ingot as to affect its whole mass. 75

The duration of immersion in any case has to be such that recalescence does not take place in the open air after the ingot has been removed from the liquid, before it is returned to the soaking pits, and if 80 they are taken from the soaking pit to the bath by reason of insufficiency of plant or other causes preventing their being treated direct from the molds, then they should be immersed at above a temperature of 800° 85 C. When thus treated from the soaking pit they should preferably be allowed first to cool slightly in such a way that the exterior is colder than the interior, as is the case with ingots direct from the mold. 90

The liquid of the bath should preferably be at a temperature of between 110° and 120° F. and there must be a sufficient quantity of the liquid to provide a thick layer all around the ingot. 95

It has heretofore been proposed to treat steel with gas, fluids, or solids in order to introduce hydrogen thereinto and such processes have been applied to high carbon and low carbon steel; it has furthermore been proposed to immerse billets in various liquid compounds but difficulty has arisen from cracking of the billets and other undesirable results. It is found that if the steel be taken in ingot form and treated by the process of this invention, it is in a form that is more favorable to such treatment than any heretofore employed and ingots can be treated containing 1.4% of carbon and the thus treated steel can be rolled without cracking. 100 105 110

Moreover, it is found that an ingot of 0.5% carbon steel treated according to this invention produces a steel approximately as hard as 0.7% carbon steel treated in the form of 5 billets.

The general effect of this process is to enhance the toughness of the steel and its ductility. The process is applicable, with advantageous results, to alloy steels, such, for 10 example, as nickel steel.

What I claim as my invention and desire to secure by Letters Patent is:—

1. The process of making steel comprising the steps of casting an ingot, stripping the 15 mold therefrom while the interior of the ingot is still molten, submerging the stripped ingot as quickly as possible and before its interior has set solid, completely beneath the surface of an aqueous bath and keeping 20 the ingot thus submerged long enough to prevent it from recalescing at its surface when removed from the bath.

2. The process of making steel comprising the steps of casting an ingot, stripping the 25 mold from the ingot while the interior is still molten, placing the ingot in a soaking pit in which the temperature is such as to prevent the interior of the ingot from setting

quickly, removing the ingot from the soaking pit before the interior of the ingot has 30 ceased to be fluid, then plunging the ingot in an aqueous bath to quickly solidify the metal and retaining the ingot in the bath long enough to cool it sufficiently to prevent it from recalescing in the open air when removed. 35

3. The process of making steel comprising the step of casting an ingot, stripping the mold therefrom as soon as the surface is hardened sufficiently to permit it to be 40 stripped, placing the ingot in a soaking pit in which the temperature is sufficiently high to prevent the interior of the ingot from setting quickly, removing the ingot from the pit while the interior is still fluid, allowing 45 the ingot to cool slightly to form a cool skin, then plunging the ingot while its interior is still fluid into an aqueous bath to quickly solidify the metal and retain it in the bath long enough to cool it sufficiently to prevent 50 it from recalescing in the open air when removed.

In testimony whereof I have signed my name to this specification.

CHARLES DEAR.

Copies of this patent may be obtained for five cents each, by addressing the "Commissioner of Patents, Washington, D. C."